

## UNITED STATES PATENT OFFICE

2,108,808

TRANSPARENT MATERIALS AND METHOD  
OF MAKING SAME

**Theron G. Finzel and Donald E. Drew, Kenmore,  
N. Y., assignors, by mesne assignments, to E. I.  
du Pont de Nemours & Company, Wilmington,  
Del., a corporation of Delaware**

No Drawing. Application June 26, 1934,  
Serial No. 732,442

17 Claims. (Cl. 91—68)

This invention relates to transparent paper, which is preferably also moistureproof, and also to a method of producing the same.

Since the advent of widespread use of moisture-proof transparent regenerated cellulose sheeting for wrapping foodstuffs, cigarettes, cigars, etc. for the purpose of protecting these various products from dust, air and moisture, while still permitting complete visibility thereof, many attempts have been made to produce a transparent and preferably also moistureproof paper. Most of the investigations have been directed to the production of an improved glassine paper. However, even the improved glassine papers do not possess the glass-clear transparency of regenerated cellulose sheeting. A certain haziness, apparent on wrapped articles, as the dulling of bright colors, always exists in the glassine-type paper. Another detrimental and undesirable property of glassine paper is its inherent brittleness, that is, its tendency to rupture at sharp folds or at the corners of packages. This is apparent in the film as white spots or lines.

We have found that we can produce a transparent paper by impregnating a highly calendered tissue paper, preferably also containing a wetting agent, with an impregnant, hereinafter more fully explained, which completely fills all the air spaces and voids in the paper. When a moistureproof product is desired, the transparentized paper is coated or impregnated with a moistureproofing lacquer.

It is, therefore, an object of this invention to provide a transparent and preferably also moistureproof paper.

Another object of this invention is to provide a method of producing a transparent and preferably also moistureproof paper.

Other objects will become apparent from the following description and appended claims.

The instant invention contemplates impregnating paper with a substantially transparent water-soluble material having an index of refraction substantially the same as that of the cellulose fibers. When a moistureproof product is desired, the impregnated material, after the impregnant has been fixed in any convenient manner, is thereafter coated with a selected moistureproof composition. The final product is highly transparent, clear, flexible, non-tacky, and possesses good surface slip. It is admirably suited for use as a wrapping tissue.

In the preferred embodiment of the invention, the paper, prior to impregnation, is super-calendered. Also, in the preferred form of the in-

vention, there is incorporated in the paper, prior to the calendering operation, a wetting agent, such as soap, as explained fully in copending application Serial No. 732,440, filed June 26, 1934.

The transparentizing impregnant should completely fill the voids, spaces, etc. in the paper and fibers thereof. This can be accomplished by any convenient procedure. The paper may, for example, be passed through an aqueous solution containing the impregnant, and the excess solution removed in any well-known manner, such as allowing the excess solution to drain off the paper or removing the excess by squeeze rolls, doctor knives, metering rolls, etc. The desired amount of solution containing the impregnant may also be applied by means of transfer rolls, buffers, brushes, etc. The impregnation with the transparentizing medium may be facilitated by subjecting the paper to vacuum before, during or after the application of the impregnating solution; by subjecting the paper to pressure while it is in contact with the impregnating solution; by the proper maintenance of temperature; or by any suitable combinations of these conditions.

The impregnating material contemplated by the instant invention is of such a nature that it gives the desired extreme flexibility and toughness. The transparentizing impregnants generally are themselves closely related to cellulose in optical properties. Thus, the thoroughly impregnated paper amounts to a continuous cellulose film. Due to the nature of the impregnants and the mode of application thereof, bonding between the cellulose of the paper and the impregnant is exceedingly strong and softening is mutual.

It is desirable that the solutions of the transparentizing impregnants be moderately fluid in concentrations of about 15%. It is, however, to be understood that it is not to be implied that the instant process cannot be worked with viscous solutions, since some materials which are so viscous as to be almost pasty will impregnate paper quite thoroughly though slowly. There, however, appears to be a relationship between viscosity and a tendency for the impregnant to shrink during drying. Generally, the higher the viscosity at one concentration, the greater the tendency for shrinkage. This excessive shrinkage has an undesirable effect because the solids of the solution tend to pull away from the paper fibers during drying, leaving the film in a spotty or hazy condition. Moreover, the shrinkage is sometimes strong enough to actually break the water-weakened paper.

5

10

15

20

25

30

35

40

45

50

55

56

In so far as the instant invention is concerned, it is to be understood that the impregnating composition may consist of a single compound or a plurality of ingredients dissolved in an appropriate liquid vehicle, such as water, water and alcohol, water and acetone, etc. For example, when an impregnant consists of a plurality of solid ingredients, one component thereof, when used alone, may give highly viscous solution and 5 be of no value for transparency, but when modified by the other components may give a composition which gives the desired effect. The preferred impregnating materials are those which are soluble in water to give practically clear solutions and which, when dry, give clear films. But, as will be explained hereafter, it is not essential that this be so. The preferred impregnants are also those which, when applied to paper and fixed thereon, leave the paper in a sufficiently non-tacky state, so that the impregnated film will not stick to itself when wound up. When the transparent paper is to be given a subsequent coating, such as when the product is to be rendered moistureproof, non-tackiness is of no 25 material importance.

As illustrative examples of the impregnating transparentizing materials contemplated by the instant invention may be mentioned the water-white variety of water-soluble or partly water-soluble substances, such as starch in various stages of deaggregation; thin boiling sizing starches, dextrin; oxidized starches; brewer's body syrups; chlorine-treated starches and other starches hydrolyzed by various means; starch 30 esters and ethers, such as starch acetate to varying degrees of acetylation up to insolubility in alcohol-water or acetone-water mixed solvents; wholly water-soluble gums, including sugar aldehyde, urea-formaldehyde and hydrolyzed vinyl 35 acetate resins; or sugars, such as cane sugar or hydrogenated sugars; sorbitol; various types of degraded or hydrolyzed celluloses, such as hemi-cellulose or cellulose precipitated from concentrated sulphuric acid solutions or derivatives of 40 various celluloses which are soluble in water or water-alcohol, such as methyl cellulose, glycol cellulose or acetates of degraded cellulose. These materials may be used alone or in combination with each other or in combination with other substances, for example, substances which soften 45 either or both the cellulose and transparentizing impregnants. As illustrative examples of such softeners may be mentioned glucose, glycerol, glycol or derivatives thereof; soluble oils, such as sulphonated castor oil and hydroxy fatty acids 50 and their salts or esters. These softeners in many cases serve for purposes other than merely flexibilizing films, for example, they may prevent spottiness of the film; they may increase 55 speed and thoroughness of impregnation; they may increase the transparency of the dry impregnated base, either by elimination of a natural haziness of one of the components of the impregnants or by changing the index of refraction of the composition to more nearly that of the cellulose fibers.

The quantity of transparentizing impregnant incorporated in the paper may vary within wide limits, depending upon the characteristics of the 60 ultimate product. Satisfactory results have been secured when the impregnant constitutes approximately 10% to 30%, by weight, of the paper.

The transparentizing impregnant may be incorporated in the paper at practically any stage 75 of the paper-making operation, such as in the

beater, on the wire, at the presses, or at any other convenient operation. In the preferred embodiment of this invention, the transparentizing impregnant is applied in an operation subsequent to the manufacture of paper, that is, to 5 a finished paper.

In the preferred embodiment of the invention, the paper base is of the thin, porous type and has the following characteristics:

1. Free from opaque filling material. 10
2. Substantially free from water-resisting sizes.
3. Has inherently transparent fibers.
4. Has a relatively smooth surface, such as may be obtained by super-calendering.
5. Is relatively compact, that is, of high solid 15 fraction.
6. Of low basis weight, not over about 20 pounds, 24" x 36", 500 sheet ream.

Though the process is most readily applied to a 20 porous paper, such as super-calendered tissue, it can also be used on non-porous paper, such as thin glassine paper, since by the process the non-porous papers are expanded by the aqueous 25 impregnating solution to such an extent that impregnation may be absolutely complete. As above explained, for the best and most rapidly obtained transparency, a wetting agent, such as soap, is incorporated in the paper prior to impregnating, and preferably also prior to super- 30 calendering.

In the foregoing embodiment of the invention, aqueous solutions of the impregnants are contemplated. As an alternative procedure, the instant invention also contemplates passing the 35 paper through a bath of transparentizing impregnants kept in the fluid state by heat. After passage through the molten impregnant and the removal of the excess material from the impregnated paper by any suitable means, the impregnant is solidified in any convenient manner, such as chilling. It is, of course, understood that this procedure is not limited to any precise manner of application, since any procedure and means will suffice as long as there is applied to 40 the paper a uniform and controllable amount of the molten impregnant. In some cases it is not even necessary to maintain the impregnant in a liquid state until impregnation is complete. Impregnation may proceed even after chilling. 50 This alternative procedure of using molten impregnants possesses the advantage that inexpensive and less complicated equipment can be used. Also, an impregnant that gives the paper a relatively tacky surface can be used without 55 very great trouble, since the impregnated paper may be surfaced, without the tacky paper ever coming into contact with any supporting mechanism, with a non-tacky coating.

As illustrative examples of substances which can be used in the molten condition may be mentioned glucose, sugar, sorbitol, sugar aldehyde resin, acetone formaldehyde resin, or any other material having similar melting and solvent 65 properties. It is desirable that the materials melt at a temperature below the charring point thereof and be relatively fluid at temperatures below the point where the paper is harmed or appreciably embrittled. This temperature for 70 the most part is below 120° C. When the above-mentioned materials melt at too high temperatures or melt to form liquids too viscous for good impregnation, a small quantity of water may be added thereto. The amount of water added 75

is preferably limited to such an amount that the swelling of the paper is slight. Also, the quantity of added water is such that it can be evaporated while the film is yet unsupported and still produce a non-wrinkled and non-distorted film. To accomplish the removal of this small amount of added water, which is preferably reduced only to an extent at which it is in equilibrium in the impregnated paper with room conditions of temperature and humidity, there is provided a short drying chamber maintained at an elevated temperature through which the film is passed after leaving the impregnating bath and the surplus-removing devices.

15 In this alternative procedure, paper of the more porous type, such as super-calendered tissue, is preferred, because these papers are subject to the most complete impregnation in the shortest time.

20 The transparentizing impregnants hereinbefore mentioned have many advantages. Once the paper has been transparentized therewith, it may be moistureproofed by practically any known process without any detrimental effects or serious complications. The water-soluble impregnants are of such a nature that they are not substantially disturbed or altered by practically any known method of moistureproofing. Thus, the instant process, in contradistinction to other processes, does not limit the composition and methods which may be used for the application of a subsequent coating.

25 When the transparent paper hereinbefore described is to be moistureproofed, any suitable moistureproofing composition may be applied thereto. As illustrative moistureproofing compositions may be mentioned those which consist of the following ingredients in such proportions as to give thin, transparent, moistureproof, 30 non-tacky coatings:

1. Cellulose derivative, wax, and solvent;
2. Cellulose derivative, wax, plasticizer, and solvent;
3. Cellulose derivative, wax, gum, and solvent;
4. Cellulose derivative, wax, gum, plasticizer, and solvent;
5. Resin, wax, and solvent;
6. Resin, wax, plasticizer, and solvent;
7. Wax compositions.

50 Though the invention has been described in connection with the production of transparent paper, that is, plain glass-like films, the process may be modified to obtain various results, such as colored products. Colored films may be produced by dyeing the paper, by dissolving a dye in the impregnating solution or in the moistureproofing composition, or a coloring substance may be applied at any convenient stage 55 in the preparation of the transparent paper. The paper may be dyed one color and the impregnants dyed another color, whereby mottled effects are secured. The paper may be embossed or designs pressed thereinto. Additional crystallizing materials may be incorporated in the impregnant to yield frosted designs.

For the purposes of this specification and claims, we define moistureproof materials as 60 those which, in the form of continuous, unbroken sheets or films, permit the passage of not more than 690 grams of water vapor per 100 square meters per hour, over a period of 24 hours, at approximately  $39.5^{\circ} \text{C.} \pm 0.5^{\circ} \text{C.}$ , the relative humidity of the atmosphere at one side of the film

being maintained at least at 98% and the relative humidity of the atmosphere at the other side being maintained at such a value as to give a humidity differential of at least 95%.

5 Moistureproofing coating compositions are defined as those which, when laid down in the form of a thin, continuous, unbroken film applied uniformly as a coating with a total coating thickness not exceeding 0.0005" to both sides of a sheet of regenerated cellulose of thickness approximately 0.0009", will produce a coated product 10 which is moistureproof.

15 For the purposes of experimental tests, especially for those materials adaptable as coating compositions, moistureproof materials include 15 those substances, compounds or compositions which, when laid down in the form of a continuous, unbroken film applied uniformly as a coating with a total coating thickness not exceeding 0.0005" to both sides of a sheet of regenerated cellulose of thickness approximately 0.0009", will produce a coated sheet which will permit the passage therethrough of not more than 690 grams of water vapor per 100 square meters per hour over a period of approximately 24 hours, at a 20 temperature of  $39.5^{\circ} \text{C.} \pm 0.5^{\circ} \text{C.}$  (preferably  $39.5^{\circ} \text{C.} \pm 0.25^{\circ} \text{C.}$ ), with a water vapor pressure differential of 50-55 mm. (preferably  $53.4 \pm 0.7$  mm.) of mercury. For convenience, the number of 25 grams of water vapor passed under these conditions may be referred to as "the permeability value". An uncoated sheet of regenerated cellulose having a thickness of approximately 0.0009" 30 will show a permeability value of the order of 35 6900.

From the foregoing, it is apparent that under the conditions set forth, a moistureproofed regenerated cellulose sheet is capable of resisting the passage of moisture or water vapor therethrough at least ten times as effectively as the 40 uncoated regenerated cellulose sheet.

In order to more fully explain the nature of the instant invention, the following illustrative examples are set forth:

#### Example I

(A) A thin porous sulphite tissue between 13 pounds and 18 pounds basis weight (24 x 36-500) is treated with the following solution consisting of the ingredients in approximately the proportions set forth:

|                   | Per cent by weight |
|-------------------|--------------------|
| Ammonium oleate   | 1.9                |
| Water             | 21.0               |
| Denatured alcohol | 77.1               |
|                   | 53                 |
|                   | 100.0              |

The excess soap solution is removed by means of squeeze rolls and the wet tissue is passed over dryer rolls. The drying is continued until the tissue feels distinctly moist (10% to 15% moisture). The damp tissue is passed through a supercalender stack, the rolls of which are cooled. This is followed by a second super-calendering operation in which heated rolls are used. If desired, these calendering operations may be combined, as by using a stack in which one-half the rolls are cooled, the other heated. As the tissue 60 emerges from the hot calender rolls, it is dry and has a fine finish. While its solid fraction has been considerably increased, the calendered paper still retains a good proportion of its absorptiveness.

The super-calendered tissue is then treated with a transparentizing composition consisting of:

|                  | Per cent by weight |
|------------------|--------------------|
| 5 Starch acetate | 20                 |
| Glycerol         | 6                  |
| Water            | 74                 |
|                  | 100                |

- 10 The starch acetate is prepared by refluxing corn starch with equal parts of glacial acetic acid and acetic anhydride for 1 hour. The starch, acetylated to about 12% acetyl content, is filtered, washed free of acid with methanol, and dried. The dried product is used in the above composition. Small amounts of acid catalysts, such as sulphonic acids, may be added in the starch acetate preparation to facilitate acetylation and to reduce the viscosity of the product.
- 15 20 The starch acetate is first dissolved by making a smooth paste of the starch acetate with equal parts of water, then adding the remainder of the water and glycerol and heating the whole solution nearly to boiling. The solution prepared will be slightly viscous and very slightly milky.

25 30 In preparing the above composition, the starch acetate is applied to the paper by immersing the paper into the solution held at 20° C. to 70° C. The excess is immediately removed by passing the paper between squeeze rolls or through scraper rods. Sufficient solution is left on the paper so that when the water is evaporated about 20 pounds to 30 pounds of impregnant to 100 pounds of paper remain. After removing the excess solution, the paper is carried over cold rolls for a sufficient period of time to allow thorough impregnation. This time is usually about 5 seconds to 10 seconds. The paper is then passed over hot rolls to evaporate the water, and the dried film is wound up.

35 40 The paper thus produced is transparent, free from any white haze or spottiness, glossy, non-tacky, and, when in equilibrium with room humidity, of exceptional flexibility and toughness.

45 (B) The transparent flexible product of Example I(A) is coated with a moistureproofing lacquer consisting of the following composition:

| Solids              | Per cent by weight |
|---------------------|--------------------|
| Nitrocellulose      | 50                 |
| Gum dammar          | 34                 |
| Tricresyl phosphate | 12                 |
| 55 Paraffin wax     | 4                  |
|                     | 100                |
| Solvents            | Per cent by weight |
| Ethyl acetate       | 62                 |
| Toluene             | 27                 |
| Alcohol             | 9                  |
| Butyl acetate       | 2                  |
|                     | 100                |
| 65 Solids content   | 15                 |

70 The transparent film is passed through the above lacquer, held at 35° C. to 45° C. and then passed through knives which remove all but a thin uniform layer of lacquer. The film is then passed into a chamber held at 60° C. to 100° C. for such a time as is necessary to evaporate the lacquer solvents. If any considerable amount of moisture is lost from the base film during the

drying operation, the coated paper is conducted through a humidifying chamber maintained at 40° C. to 70° C. and 60% to 95% relative humidity to restore the film to its normal moisture content, and the film wound up.

75 The product obtained is moistureproof, transparent, non-smeary, non-tacky, glossy and free from spots or white haze. Furthermore, its flexibility and toughness is such that it can be creased and folded without the appearance of 10 white lines.

(C) The transparent, flexible film obtained in Example I(A) is passed through a melt of the following composition:

| Per cent by weight   |    |
|----------------------|----|
| White paraffin wax   |    |
| Refined carnauba wax |    |
| Rubber (crepe)       |    |
|                      |    |
| 100                  | 20 |

The paper is passed through the molten composition and then through a set of two doctor knives on each side of the film by which all but a uniform layer of composition is scraped from the film. About 5 pounds of the wax composition to 100 pounds of the transparent film are applied.

25 30 The product obtained is moistureproof, transparent, glossy, free from white haze, non-smeary, and sufficiently tough and flexible to withstand drastic flexing and creasing without showing undesirable white lines.

#### Example II

(A) The same calendered paper as in Example I(A) is impregnated and dried exactly as in that example, but using the following impregnating solution:

| Per cent by weight |    |
|--------------------|----|
| Starch acetate     |    |
| Sorbitol           |    |
| Water              |    |
|                    |    |
| 100                | 45 |

The film obtained is glossy, non-tacky, free from white spots or haze, and of exceptional flexibility. Its transparency is somewhat better than that of Example I(A), since the refractive index of the impregnant is more nearly that of the cellulose.

(B) A moistureproof, transparent, and flexible film is produced from the product of Example II(A) by coating it with the following composition and by the procedure outlined in Example I(B):

| Per cent by weight      |    |
|-------------------------|----|
| Pyroxylin               |    |
| Gum dammar              |    |
| Dibutyl phthalate       |    |
| Paraffin (62° C. M. P.) |    |
| Zinc stearate           |    |
| Toluol                  |    |
| Ethyl acetate           |    |
| Ethyl alcohol           |    |
| Acetone                 |    |
|                         |    |
| 100.00                  | 70 |

A product is obtained which is equal to that of Example I(B) in strength and flexibility and is superior in transparency and clarity.

(C) The same calendered paper as in Example I(A) is treated with the following impregnating solution:

Per cent by weight

|                                              |    |
|----------------------------------------------|----|
| 5 Starch acetate (high acetyl content) ----- | 20 |
| Sorbitol -----                               | 10 |
| Water -----                                  | 30 |
| Denatured alcohol -----                      | 40 |

10 100

The paper is passed through the impregnating solution and then through squeeze rolls to remove the excess solution. When impregnation is complete, the paper is passed over hot dryer rolls and the paper dried.

15 There are some advantages in using the higher starch acetate. The above solution is usually somewhat less viscous than previous starch acetate solutions and, therefore, it more rapidly penetrates or impregnates the paper; the starch acetate of higher acetyl content usually results in a more transparent film; the use of alcohol in the impregnating solution decreases the softening power which water has on the thin tissue, so that there is less likelihood of breakage in the impregnating solution.

20 The product obtained is very transparent and glossy and of excellent flexibility. It may be moistureproofed with any convenient composition and means.

*Example III*

(A) The same paper as in Example I(A) is given the same treatment as in Example I(A), except that the following impregnating solution is used:

Per cent by weight

|                     |    |
|---------------------|----|
| Sizing starch ----- | 20 |
| Glucose -----       | 20 |
| Water -----         | 60 |

100

45 The sizing starch used here is a hydrolyzed corn starch commercially produced by the Corn Products Refining Company and sold as Amidex #130.

50 The product obtained, while being exceptionally tough and flexible, has a somewhat hazy and dull appearance, is of rather poor transparency, and is somewhat tacky. Instead of winding up the film in this condition after drying, it is passed directly into a moistureproofing lacquer and coated as in Example I(B).

55 The moistureproof product obtained will possess its original flexibility and toughness and in addition will have imparted to it by the coating procedure a good degree of transparency and gloss, and will be free from any haziness or spottiness.

60 (B) A transparent, flexible film, similar to that obtained in Example II(A), except for a slightly greater degree of tackiness, is obtained if the calendered sulphite tissue, instead of being impregnated with a starch acetate solution, is impregnated with a solution of the following composition:

Per cent by weight

|                          |      |
|--------------------------|------|
| 70 Oxidized starch ----- | 20.0 |
| Sorbitol -----           | 7.5  |
| Glycerol -----           | 2.5  |
| Water -----              | 70.0 |

75 100.0

Somewhat highly oxidized starch, such as a thin British gum, may be used. The product obtained, while being transparent and flexible, is too tacky to be wound up on itself. Consequently, it is desirable to apply immediately any suitable moistureproofing composition by which a transparent and flexible film is obtained and through which tackiness is eliminated.

*Example IV*

10

(A) A tissue between 13 pounds and 18 pounds basis weight ( $24 \times 36 = 500$ ) is passed through a calender, preferably in a slightly moistened condition.

15 The calendered paper is impregnated with a 50% sorbitol solution in water by supplying about 10 pounds of solution to 100 pounds of paper to each side of the film with suitable hoppers. The paper is passed over cold rolls 20 until impregnation is complete, and then over hot rolls to expel the water. Without winding the film up, it is immediately coated with a moistureproofing lacquer following the procedure in Example I(B). The product obtained will be 25 moistureproof, free from haze or spots, transparent and very flexible.

(B) A good grade of glassine, 20 pounds basis weight, is passed through a 50% sorbitol water solution and then through squeeze rolls to remove all but about 15 pounds to 30 pounds of solution, to 100 pounds of glassine. The paper is rolled up and allowed to stand for 1 to 5 hours. During the time of standing, a limited amount of swelling proceeds (the full swelling 30 power of the water is limited by the high concentration of sorbitol) and the sorbitol slowly penetrates into the film, displacing the entrapped air. When the glassine has been sufficiently 35 impregnated, it is dried on dryer rolls or other suitable means, and the tacky transparent film passed through a moistureproofing lacquer as outlined in Example I(B).

40 The product obtained will be very transparent, exceptionally flexible and tough, glossy, non-smeary and moistureproof, and will be free from the normal glassine haze and spottiness. Had the sorbitol treatment been omitted and the glassine simply coated with a moistureproofing lacquer, both transparency and flexibility would 45 have been markedly less and the original hazy, spotty appearance of the glassine not materially altered.

50 (C) The same calendered sulphite tissue as in Example I(A) is treated with a water-soluble resin solution of the following composition:

|                |    |
|----------------|----|
| Resin -----    | 30 |
| Glycerol ----- | 5  |
| Water -----    | 65 |

100

65 The resin used in this example is the condensation product of acetone and formaldehyde, a slightly yellow, slightly brittle resin. The resin solution is applied, the water evaporated, and the product coated with a lacquer as in Example IV(A). A glossy, non-smeary, moistureproof product of high transparency and great flexibility is obtained.

*Example V*

70 (A) The same calendered tissue as in Example I(A) is impregnated as follows: The paper is passed through a tank containing sorbitol which 75

has been heated sufficiently to be a slightly viscous liquid, then out of the tank and through doctor knives so adjusted as to remove all but about 10 pounds of sorbitol for 100 pounds paper.

5 It is preferable that the surface of the paper be completely covered with a thin film of the sorbitol. The sorbitol is kept in a molten condition until the paper is thoroughly impregnated and is then cooled by a blast of cold air or is simply 10 allowed to cool of itself. The impregnated paper is passed between suitable hopper lips or over transfer rolls by which a molten wax composition similar to that of Example I(D) is uniformly applied to both sorbitol surfaces. If the original 15 sorbitol bath contains the proper amount of moisture, it is not necessary to further humidify the film.

The product obtained is very glossy and transparent, moistureproof, non-tacky and non-smearable, and of exceptional flexibility.

(B) The same paper is given the same treatment as in Example IV(A), except that a molten bath of the following composition is substituted for the sorbitol:

|            | Percent by weight |
|------------|-------------------|
| Glucose    | 70                |
| Corn syrup | 30                |
|            | 100               |

30 With this composition it is not necessary to allow impregnation to proceed fully to completion before chilling the molten composition, since impregnation with this composition proceeds slowly, 35 even at room temperature. The product will be similar in all respects to that of Example V(A).

(C) The same paper as in Example I(A) is impregnated with:

|          | Percent by weight |
|----------|-------------------|
| Dextrin  | 40                |
| Sorbitol | 40                |
| Water    | 20                |
|          | 100               |

45 The paper is passed through this solution held at a sufficiently high temperature to be fluid, thence out of the solution and through suitable doctor knives or squeeze rolls to remove the excess. After removal of the excess solution, the film is passed through a short drying chamber held at an elevated temperature, by which the water is evaporated to such a content as to be in equilibrium with room humidity. The impregnated paper is then passed through a moisture-proofing lacquer and coated by the same procedure as outlined in Example I(B).

The product obtained is non-tacky, non-smearable, glossy and of very good transparency 60 and flexibility.

Though the invention has been particularly described in connection with transparent and moistureproof paper, the principles thereof are equally applicable to non-moistureproof, such as, for 65 example, waterproof, and transparent paper.

Since it is obvious that various changes and modifications may be made in the above description without departing from the nature or spirit thereof, this invention is not restricted thereto 70 except as set forth in the appended claims.

We claim:

1. A transparent moistureproof material comprising paper containing a wetting agent and having its voids and spaces substantially completely filled with a water-soluble impregnant

and thinly coated with a transparent moisture-proofing composition, said impregnant being present in an amount of 10% to 30%, by weight, of the paper.

2. A transparent moistureproof material comprising highly calendered porous paper containing a wetting agent and having its voids and spaces substantially completely filled with a water-soluble impregnant and thinly coated with a transparent moistureproofing composition, said 10 impregnant being present in an amount of 10% to 30%, by weight, of the paper.

3. A method of making a transparent material which comprises incorporating a non-volatile wetting agent in paper, highly calendering the 15 paper, impregnating said paper to substantially completely fill the spaces and voids therein with a water-soluble transparentizing agent whereby the paper is transparentized, and finally applying a transparent, moistureproof coating to the 20 transparentized paper.

4. A method of making a transparent material which comprises incorporating a non-volatile wetting agent in paper, highly calendering the 25 paper, impregnating said paper to substantially completely fill the spaces and voids therein with an aqueous solution containing a water-soluble transparentizing agent, evaporating the water whereby the paper is transparentized, and finally applying a transparent, moistureproof coating 30 to said transparentized paper.

5. A method of preparing transparent material which comprises incorporating a non-volatile wetting agent in paper, highly calendering the 35 paper, impregnating said paper to substantially completely fill the spaces and voids therein with a water-soluble transparentizing agent in the molten state, setting the impregnant whereby the paper is transparentized, and finally applying a transparent, moistureproof coating to the 40 transparentized base.

6. A method of making a transparent material which comprises incorporating a non-volatile wetting agent in paper, highly calendering the 45 paper, impregnating said paper to substantially completely fill the spaces and voids therein with a water-soluble substance selected from the class which consists of starches and starch compounds; and hydrolyzed vinyl resins; whereby the paper is transparentized, and applying a transparent 50 moistureproofing coating.

7. A transparent material comprising highly calendered paper containing a wetting agent and having its voids and spaces substantially completely filled with a water-soluble substance selected from the class which consists of starch and starch compounds, said substance being present in an amount of 10% to 30% by weight of the 55 paper, said paper being thinly coated with a transparent moistureproof composition.

8. A transparent moistureproofing material comprising paper containing a wetting agent distributed throughout its mass and having its spaces and voids substantially completely filled with a transparentizing water-soluble substance, where- 60 by said paper is transparentized.

9. A transparent moistureproofing material comprising paper containing a wetting agent distributed throughout its mass and having its spaces and voids substantially completely filled with a 65 transparentizing water-soluble substance where- by said paper is transparentized, said paper being thinly coated with a transparent moistureproofing composition.

10. A transparent material comprising highly 75

5 calendered paper containing a wetting agent distributed throughout its mass and having its spaces and voids substantially completely filled with a water-soluble substance selected from the class which consists of starch and starch compounds.

10 11. A transparent material comprising highly calendered paper containing a wetting agent distributed throughout its mass and having its spaces and voids substantially completely filled with starch acetate.

15 12. A transparent material comprising highly calendered paper containing a wetting agent distributed throughout its mass and having its spaces and voids substantially completely filled with chlorine-treated starch.

20 13. A transparent material comprising highly calendered paper containing a wetting agent distributed throughout its mass and having its spaces and voids substantially completely filled with oxidized starch.

25 14. A transparent material comprising highly calendered paper containing a wetting agent distributed throughout its mass and having its spaces and voids substantially completely filled with a water-soluble substance selected from the class

which consists of starch and starch compounds, said paper being thinly coated on each side thereof with a transparent moistureproof composition.

15 15. A transparent material comprising highly calendered paper containing a wetting agent distributed throughout its mass and having its spaces and voids substantially completely filled with starch acetate, said paper being thinly coated on each side thereof with a transparent moisture-proof composition. 5

10 16. A transparent material comprising highly calendered paper containing a wetting agent distributed throughout its mass and having its spaces and voids substantially completely filled with chlorine-treated starch, said paper being thinly 15 coated on each side thereof with a transparent moistureproof composition.

15 17. A transparent material comprising highly calendered paper containing a wetting agent distributed throughout its mass and having its spaces 20 and voids substantially completely filled with oxidized starch, said paper being thinly coated on each side thereof with a transparent moisture-proof composition.

THERON G. FINZEL. 25  
DONALD E. DREW.